

May 13, 1969

J. GALEY ET AL

3,443,806

METHOD OF USING INDUCTION FURNACES

Filed Aug. 10, 1966

Sheet 1 of 2

Fig.1



Fig.2



INVENTORS

JEAN GALEY  
GILBERT VALIN

By Young & Thompson

ATTYS

May 13, 1969

J. GALEY ET AL

3,443,806

METHOD OF USING INDUCTION FURNACES

Filed Aug. 10, 1966

Sheet 2 of 2

Fig.3



Fig.4



INVENTORS

JEAN GALEY  
GILBERT VALIN

BY Young & Thompson  
ATRYS

1

3,443,806  
**METHOD OF USING INDUCTION FURNACES**  
Jean Galey, Ville d'Avray, and Gilbert Valin, Noiserau,  
France, assignors to L'Air Liquide, Paris, France  
Filed Aug. 10, 1966, Ser. No. 597,185  
Int. Cl. C21c 5/00

U.S. Cl. 266—34

5 Claims

## ABSTRACT OF THE DISCLOSURE

A metallurgical induction furnace is operated by imposing an alternating electromagnetic field on molten metal in a crucible, and blowing fine bubbles of gas through a lower porous surface of the crucible. Among other advantages, the trapping of solid impurities against the walls of the crucible is prevented.

The present invention relates to a method of using metallurgical induction furnaces, more particularly those using a medium frequency and not employing a vacuum.

It is characterised in that an agitating gas in the form of fine bubbles is blown in at the lower portion of the crucible of the furnace, this gas supplementing and correcting the electromagnetic agitating effects.

Users of special alloys and steels are stressing more and more the need for providing metals of high quality, and more particularly for being able to rely on the uniformity of the properties of such metals.

Of these properties, purity, characterised by the absence of inclusions and homogeneity are particularly important.

In order to obtain uniformity of such properties, use is frequently made of operating under a vacuum or in a protected atmosphere.

The use of a vacuum requires a relatively expensive and complicated apparatus and does not solve all the problems. It is known more particularly that treatment under a vacuum cannot itself ensure complete decantation of solid impurities nor the total elimination of occluded gases.

More particularly, in the case of an induction furnace, the flow of the metal caused by the action of the alternating magnetic field occurs along more or less complicated paths of travel, in which descending currents are formed along the walls of the furnace. These currents, which are described more particularly in the work, "Métallurgie du fer" (Dunod, 1957, 2nd edition), pages 311-312 by L. Colombier, result in an irreversible trapping of the inclusions by the walls of the furnace. It will be appreciated that the action of the vacuum cannot by itself modify this phenomenon.

According to the present invention it has been found that it is possible to combine advantageously the effects of the electromagnetic agitation with those of the blowing in of an agitating gas in fine bubbles through at least one porous refractory element inserted in the bottom of the crucible of an induction furnace.

Tests have in fact shown the possibility of using the blowing in of gas to correct the unfavourable effects of electromagnetic agitation, whilst promoting on the other hand certain advantageous effects of this agitation, more particularly as regards the homogenisation of the alloying elements which are heavier than iron, such as tungsten, or on the contrary which are lighter than iron, when iron is the metal to be treated.

It has been found more particularly that the suitably directed blowing in of gas in fine bubbles not only enables the descending currents of liquid metal to be deflected so as to move them away from the walls of the furnace, but also makes it possible to carry towards the surface of the molten bath the solid particles which have adhered to the walls.

2

Preferably, a cover is arranged on the upper portion of the furnace crucible, this cover being provided if desired with a pipe for the introduction of inert gas. The usefulness of this cover, often very considerable, is to create above the bath an inert atmosphere emanating from the agitating gas and with which the ambient air does not mix.

In the accompanying drawings:

FIGURE 1 shows diagrammatically the flow of the metal in a conventional induction furnace.

FIGURE 2 shows diagrammatically this flow modified by the blowing in of an agitating gas according to the invention.

FIGURE 3 shows in section a portion of one form of embodiment of the invention.

FIGURE 4 is a graph showing the consumption of agitating gas in various cases.

In FIGURES 1 and 2 induction furnaces have been shown which are open to the ambient air and whose crucible 1 is surrounded by a heating solenoid 2 through which flows an alternating current at medium frequency (of about 500 to 2000 cycles per second).

The furnace in FIGURE 1 is a typical example of the known art whereas the furnace shown in FIGURE 2 has had the improvement which forms the subject of the present invention applied to it.

In the furnace shown in FIGURE 1 currents 3 flow in the liquid metal as follows:

On the one hand about an equatorial plane of symmetry HH', situated substantially halfway up the height 30 of the bath; and on the other hand about a vertical axis of symmetry XX' substantially coincident with the vertical axis of the crucible.

At the upper portion of the bath, these currents 3 flow downwardly along the walls of the crucible, with the result 35 that there is an irreversible trapping of the solid impurities of the metal, which are constantly kept in contact with the walls of the crucible, mainly in the lower portion of the said crucible.

In FIGURE 2 the induction furnace is provided with a 40 porous refractory plug 4 inserted in the lining of the crucible bottom. A conduit 5 is used for introducing a gas under pressure through the porous plug. This gas, entering into the metal at the bottom of the crucible, gives rise to a rapid ascending current 6 constituted by an emulsion of 45 gas in the metal, in which the gas is dispersed in a multitude of fine bubbles each of which is capable of fixing, by adsorption, one or more solid particles and of entraining even those which have adhered to the walls before the blowing-in operation has commenced. It is to be noted 50 that the current 6 is much more rapid than the currents 3 which are produced by the alternating magnetic field.

On the other hand, the blowing in of an inert gas in 55 fine bubbles through the bottom of the furnace promotes the release of occluded gases since each bubble of inert gas constitutes a micromedium in which the occluded gas is initially at a zero partial pressure, so that the occluded gases tend to issue from the metal and pass into the bubble, until the partial pressure is balanced. The total 60 surface of the bubbles is greater in proportion as their diameter is smaller, and this factor plays an important part in the decantation of the solid impurities and the elimination of occluded gases.

Another favourable effect of blowing in gas is that it 65 opposes the concentration of the heavy additions, such as ferrotungsten, in the bottom of the furnace, and the concentration of the light additions in the upper layers.

Blowing in may take place either whilst electromagnetic agitation is taking place or whilst the electromagnetic arrangement is inoperative.

Finally, a subsidiary result of considerable interest is that the metal is protected not only during its prepara-

tion but until it is poured when the furnace is tipped, owing to the presence of a layer of inert gas covering the surface of the bath. This surface is thus protected from contact with the atmosphere.

The blowing in of inert gas through the bottom ensures that this gas, after having passed through the bath of molten metal, covers the entire surface of the bath; in this respect, this method of blowing in is reliable and more advantageous than a method consisting in using lances or nozzles directed towards the surface of the bath, which are consequently capable of entraining air against the said surface by an ejector effect.

Consequently the blowing in of inert gas through the crucible bottom achieves, in conjunction with electromagnetic agitation, an improvement in the efficiency of readily slagable additions (titanium, aluminum, calcium etc.); in fact, in current induction furnace practice, an often very considerable proportion of these additions is burned in contact with air before there is a possibility of being incorporated in the liquid metal.

The invention also relates, as a novel apparatus, to an induction furnace particularly of a medium-frequency type the bottom of which is provided with one or more porous plugs arranged in such a manner as to permit the blowing in of gas under the conditions defined hereinbefore.

The use of a porous plug permits of introducing the gas at the lower portion of the metal bath, contrary to what occurs when using a lance which enters the metal bath, and a lance is also much more difficult to protect from the heat of the bath and the corrosive action thereof.

Furthermore, the improvement provided by the invention, which consists in making the gas agitation and the electromagnetic agitation effects supplement one another, can considerably widen the field of application of the electric furnace, more particularly by making it possible to agitate the metal in contact with the slag in this furnace, in the manner similar to that used in the Ugine-Perrin process.

The agitation may be applied more particularly to desulphurisation and dephosphorisation operations in the induction furnace. It may also be used so as to deoxidise steels and, in operations for the production of special cast irons, so as to bring the graphite to a modular form. In these various operations, the inert gas can serve as a carrier for an active gas, for example a reducing gas, or the vapours of a relatively volatile metal such as sodium or magnesium.

FIGURE 3 represents diagrammatically and by way of a nonlimiting example, the upper portion of an induction furnace similar to that shown in FIGURE 2, in a vertical section taken through its axis.

The crucible 23 of the furnace and its induction coil 2 are arranged below a floor 30. In the bottom of the crucible, not shown, there is arranged a refractory porous plug through which an agitating gas is blown in; bubbles of this gas are shown at 32, 34 for example, in the metal bath 36 to be treated. A cover closes the upper opening of the crucible except for its pouring spout 38 if appropriate. This cover is made of sheet metal 40 lined internally with refractory material 42. It is supported on the crucible. A seal is provided if appropriate by a refractory mortar 44.

The cover prevents the oxidation of the metallic bath by the ambient air. It creates an inert atmosphere between it and the bath, emanating from the agitating gas. It may be advantageous to provide a pipe 46 through which an inert gas is injected so as to create the protective atmosphere more quickly and to maintain it more

satisfactorily. The cover may be designed so as to close the pouring spout also.

Experience has shown that the rate of flow of agitating gas is to be between 0.2 and 2 litres per minute per square centimetre of porous plug surface in contact with the molten metal to be treated. If the flow rate is too low, there is inadequate agitation, and the provision of the porous plug and its gas supply is not worthwhile. If the flow rate is too high, the effectiveness of the gas is much less.

In cases where the agitating gas is used also to degasify the metal, its consumption depends more particularly on the degree of degasification which it is desired to achieve, and the output rate. This consumption is generally between 1 and 15 m.<sup>3</sup> of gas per ton of metal, preferably between 2.3 and 10 m.<sup>3</sup>, all gas volumes herein being given at standard temperature and pressure.

FIGURE 4 relates to the dehydrogenation of steel by the injection of argon. It shows how the quantity of gas consumed varies, this being plotted as ordinates in m.<sup>3</sup> per ton, as a function of the specific flow rate, which is plotted as abscissae and is counted in litres per minute and per cm.<sup>2</sup> of blowing in surface at the plug.

Each of the curves relates to a specific dehydrogenation of the treated steel:

20 The curve 48 relates to a reduction of from 5 to 3 cm.<sup>3</sup> of hydrogen per 100 g. of steel.

The curve 50 to a reduction of from 4 to 2 cm.<sup>3</sup> per 100 g.

25 The curve 52 to a reduction of from 4 to 1.5 cm.<sup>3</sup> per 100 g.

It will be seen from these curves that it is advantageous to use low flow rates, but limits are set to this by the slowing down of the operation.

30 What we claim is:

1. A method of treating molten metal in a metallurgical induction furnace, comprising imposing an alternating electromagnetic field on molten metal in a crucible at a medium frequency of about 500 to about 2,000 cycles per second, blowing fine bubbles of inert gas through a lower porous surface of the crucible in a quantity about 1 to about 15 cubic meters at standard temperature and pressure per ton of molten metal, and maintaining the pressure at the surface of the molten metal at least atmospheric.

2. A method as claimed in claim 1, and confining to the region immediately above the surface of the molten metal the inert gas that emerges from the molten metal.

3. A method as claimed in claim 2, and initially purging the said region immediately above the molten bath with said inert gas.

4. A method as claimed in claim 1, the flow rate of said gas being from about 0.2 to about 2 liters per minute and per square centimeter of said porous surface that contacts the molten metal.

5. A method as claimed in claim 1, said inert gas being supplied in a quantity about 2.3 to about 10 cubic meters under standard temperature and pressure per ton of molten metal.

#### References Cited

#### UNITED STATES PATENTS

- |           |         |          |
|-----------|---------|----------|
| 2,322,618 | 6/1943  | De Mare. |
| 2,956,794 | 10/1960 | Allard.  |
| 3,240,588 | 3/1966  | Finkl.   |

CHARLES J. MYHRE, Primary Examiner.